

3,829,322  
PRESSURE-SENSITIVE PHTHALIDE COMPOUND  
COPYING SHEET

Minoru Ozutsumi, Yoshihide Miyazawa, and Katsuichi Motohashi, Tokyo, and Masataka Kiritani, Shizuoka, Japan, assignors to Hodogaya Chemical Co., Ltd., Tokyo, and Fuji Photo Film Co., Ltd., Kanagawa, Japan

No Drawing. Filed Dec. 23, 1971, Ser. No. 211,757  
Claims priority, application Japan, Dec. 28, 1970,

46/119,950

Int. Cl. B41m 5/22

U.S. Cl. 117—36.8

5 Claims

### ABSTRACT OF THE DISCLOSURE

A pressure-sensitive copying sheet comprising an adsorbent solid acid and a microencapsulated color former capable of forming a distinct color when reacted with said adsorbent solid acid coated on the same or different surface of support or supports, said microcapsules containing an organic solvent having dissolved therein as a color former at least one phthalide compound represented by the following formula:



wherein R<sub>1</sub>, R<sub>2</sub>, R<sub>3</sub>, R<sub>4</sub>, X, Y and n are described hereinbelow, is disclosed.

### BACKGROUND OF THE INVENTION

#### 1. Field of the Invention

The present invention relates to a pressure-sensitive copying paper, more particularly to a pressure-sensitive copying paper having a microcapsule layer containing a novel phthalide compound as a color former.

#### 2. Description of the Prior Art

Pressure-sensitive copying papers generally comprise a transfer sheet having thereon a layer of fine capsules containing therein a solution of an electron donating colorless organic compound (hereinafter the organic compound is called the "color former") in an organic solvent, and a receiving sheet, having thereon a layer of an electron-accepting solid. A suitable binder is usually present to contain the solid.

When both sheets are put together such that the electron donating layer is brought into contact with the electron accepting layer, and local pressure is applied to the combination by handwriting or typewriting, the capsules are ruptured and the colorless color former contained in the capsules is adsorbed on the electron accepting solid, usually a solid acid, to form the color.

Pressure-sensitive copying paper systems are also known which consist of the aforesaid transfer sheet (hereinafter this sheet is called the "upper sheet") and a receiving sheet (hereinafter this sheet is called the "lower sheet") and an intermediate sheet (hereinafter this sheet is called the "middle sheet"). In these systems the middle sheet usually has coated, on opposite surfaces, a layer of microcapsules containing the color former solution and a layer of the solid acid and a binder.

As another embodiment of pressure-sensitive copying systems, there is a recording sheet which may be prepared

by coating the above described microcapsules and the adsorbent solid acid on the same surface of a support.

As the electron accepting solid material, solid acids are usually used, e.g. acid clay, attapulgite, zeolite, bentonite, kaolin, acid polymers such as phenolic resin and the like. Illustrative organic solvents for dissolving the color former are ethylene glycol, chlorobenzene, and chlorodiphenyl.

In general, Crystal Violet Lactone has widely been used as a purple-color former. Although Crystal Violet Lactone is immediately colored purple-blue when it is brought into contact with an electron-accepting solid acid, it suffers from the following disadvantages: the color exhibits poor light fastness and the purple-blue vanishes upon contact with water.

Benzoyl Leuco Methylene Blue has also been used as a blue-color former. When the color former is brought into contact with an electron accepting solid acid, a blue color having good light fastness is formed but this color former has the disadvantage that it takes a long period of time to color.

To partially overcome the above disadvantages a mixture of these color formers has been used. However, for the reasons mentioned above the color formed on pressure-sensitive copying papers using the mixture of these color formers changes gradually from purple-blue to blue and to dark blue with the passage of time.

Recently, pressure-sensitive copying sheets in which an indole-substituted phthalide compound is used as the color former were disclosed by Chao-Han Lin and Dayton in U.S. Pat. No. 3,540,911. However, the compounds described in the specification of this patent have the following disadvantages: the color density of the color obtained by the contact thereof with an electron-accepting solid acid is not high and the colored compound exhibits weak water resistance.

### SUMMARY OF THE INVENTION

According to the present invention, there is provided a pressure-sensitive copying paper containing as a color former the phthalide compound represented by the general formula



wherein R<sub>1</sub> represents a hydrogen atom, a methyl group, an ethyl group, an acetyl group, or a benzyl group; R<sub>2</sub> represents a methyl group, or an ethyl group; R<sub>3</sub> represents a hydrogen atom, a methyl group, or an ethyl group; R<sub>4</sub> represents a methyl group, or a phenyl group; X represents a methyl group, methoxy group, or an ethoxy group; Y represents a hydrogen atom, a chlorine atom, a bromine atom, or a dimethylamino group; and n is an integer from 1 to 4.

### DETAILED DESCRIPTION OF THE INVENTION

An object of the present invention is, therefore, to provide pressure-sensitive copying papers containing as a color former the phthalide compound represented by the aforesaid general formula which is immediately colored when it is brought into contact with a solid acid to provide a stable purple or blue color having excellent light fastness and water resistance.

An object of this invention is to provide pressure-sensitive copying papers which can be colored various colors by using the phthalide compound represented by the afo-

said general formula together with other known color formers.

The phthalide compounds used in this invention represented by the general formula described above may be prepared by applying the process for forming the indole substituted phthalide disclosed in the specification of U.S. Pat. No. 3,540,911.

The phthalides are conventionally prepared by the following reaction,



Thus, the phthalide compound used in this invention represented by the general formula described above may be prepared by reacting the corresponding benzophenone carboxylic acid and an indole or the corresponding benzoylindole and an aromatic amine for 1-10 hours at a reaction temperature of 50-130° C., in the presence of a condensing agent such as acetic anhydride or phosphorus oxychloride using, if necessary, a volatile inert organic solvent such as benzene, or chloro-benzene, pouring the reaction mixture in ice-cooled water or a dilute aqueous solution of an acid such as hydrochloric acid to hydrolyze the condensing agent, adding a volatile inert solvent such as benzene or chlorobenzene to extract the product, alkalinizing the reaction mixture with an aqueous solution of a basic material such as sodium hydroxide, recovering the solvent layer, and distilling away the solvent therefrom under reduced pressure.

Examples of producing such phthalide compounds used in this invention will be explained below in detail.

#### PRODUCTION EXAMPLE 1

A mixture of 2.0 g. of 1,2-dimethyl-3-(2'-carboxybenzoyl)-indole, 1.6 g. of N,N-diethyl-m-toluidine, and 14.3 g. of acetic anhydride was heated to 50-55° C. for 10 hours, with stirring, to cause the reaction. The reaction mixture was poured in 400 g. of ice-water to hydrolyze the acetic anhydride, and after adding thereto 100 g. of benzene, the pH of the mixture was adjusted to 12 by adding an aqueous solution of sodium hydroxide. The benzene layer formed was recovered by decantation and after treating the benzene layer with activated carbon, benzene was distilled off under reduced pressure. Then, by recrystallizing the residue from petroleum ether, 2.0 g. of 3-(2'-methyl-4'-diethylaminophenyl)-3-(1',2'-dimethylindol-3'-yl)-phthalide represented by the following formula



was obtained as a white color former having a melting point of 180-182° C. When a benzene solution of the

color former thus prepared was brought into contact with an acid clay layer coated on a paper, the color former immediately colored blue.

#### PRODUCTION EXAMPLE 2

A mixture of 2.0 g. of 1,2-dimethyl-3-(2'-carboxybenzoyl)-indole, 1.5 g. of N,N-diethyl-m-phenetidine, and 14.3 g. of acetic anhydride was heated to 90-95° C. for 1 hour, with stirring, to cause the reaction. Then, the reaction mixture was treated as in Production Example 1 to provide 2.8 g. of 3-(2'-ethoxy-4'-diethylaminophenyl)-3-(1',2'-dimethyl-indol-3'-yl)-phthalide represented by the following formula



as a white color former having a melting point of 215-216° C. When a benzene solution of the color former was brought into contact with an acid clay layer coated on a paper, the color former immediately colored violet-blue.

#### PRODUCTION EXAMPLE 3

To 15 g. of monochlorobenzene were added 2.0 g. of 1,2-dimethyl-3-(2'-carboxybenzoyl)-indole and 1.1 g. of N-methyl-m-anisidine and then 1.6 g. of phosphorus oxychloride was further added to the mixture.

The resultant mixture was heated to 100-105° C. for 2 hours with stirring to cause the reaction. The reaction mixture was poured in 400 g. of ice-water to hydrolyze the phosphorus oxychloride, and after adding thereto 100 g. of monochlorobenzene, the pH of the mixture was adjusted to 12 by adding an aqueous solution of sodium hydroxide. The monochlorobenzene layer formed was recovered by decantation and after treating the monochlorobenzene layer with activated carbon, monochlorobenzene was distilled off under reduced pressure. Then, by recrystallizing the residue from petroleum ether, 1.6 g. of 3-(2'-methoxy-4'-methylaminophenyl)-3-(1',2'-dimethylindol-3'-yl)-phthalide represented by the following formula



was obtained as a light-color former having a melting point of 200-202° C. When a benzene solution of the color former was brought into contact with an acid clay layer coated on a paper, the color former immediately colored violet.

#### PRODUCTION EXAMPLE 4

A mixture of 2.0 g. of 1,2-dimethyl-3-(2'-carboxy-3',4',5',6'-tetrachlorobenzoyl)-indole, 0.8 g. of N,N-dimethyl-m-anisidine, and 10.0 g. of acetic anhydride was heated to 80-90° C. for 2 hours, with stirring, to cause the reaction. Then, the reaction mixture was treated as in Production Example 1 to provide 2.0 g. of 3-(2'-methoxy-4'-dimethylaminophenyl)-3-(1',2'-dimethylindol-3'-yl)-4,

5

5,6,7-tetrachlorophthalide represented by the following formula



as a light-green color former having a melting point of 251–253° C. When a benzene solution of the color former was brought into contact with an acid clay layer coated on a paper, the color former immediately colored blue.

#### PRODUCTION EXAMPLE 5

A mixture of 2.2 g. of 4-diethylamino-2-ethoxy-5'-dimethylamino-benzophenone - 2' - carboxylic acid, 0.9 g. of 1,2 - dimethylindole, and 11.5 g. of acetic anhydride was heated to 55–60° C. for 4 hours, with stirring, to cause the reaction. Then, the reaction mixture was treated as in Production Example 1 to provide 2.2 g. of 3-(2'-ethoxy - 4' - diethylaminophenyl) - 3 - (1',2' - dimethylindol-3'-yl)-5-dimethylaminophthalide represented by the following formula



as a white color former having a melting point 193–194° C. When a benzene solution of the color former was brought into contact with an acid clay layer coated on a paper, the color former immediately colored violet-blue.

#### PRODUCTION EXAMPLE 6

A mixture of 1.2 g. of 1-methyl-2-phenyl-3-(2'-carboxy-3',4',5',6'-tetrabromobenzoyl)-indole, 0.5 g. of N,N-diethyl-m-phenetidine, and 5.0 g. of acetic anhydride was heated to 80–85° C. for 3 hours, with stirring, to cause the reaction. Then, the reaction mixture was treated as in Production Example 1 to provide 1.1 g. of 3-(2'-ethoxy-4' - diethylaminophenyl) - 3 - (1' - methyl - 2' - phenylindol-3'-yl)-4,5,6,7-tetrabromophthalide represented by the following formula



as a light-yellow color former having a melting point of 205–206° C. When a benzene solution of the color former was brought into contact with an acid clay layer coated on a paper, the color former immediately colored blue.

#### PRODUCTION EXAMPLE 7

To 15 g. of monochlorobenzene were added 2.3 g. of 4 - diethylamino - 2 - ethoxy-benzophenone - 2' - carboxylic acid, 1.0 g. of 2-methylindole and then 1.6 g. of phosphorus oxychloride was further added to the mixture. The resultant mixture was heated to 100–105° C. for 4 hours, with stirring, to cause the reaction and the

6

reaction mixture was treated as in Production Example 3 to provide 1.6 g. of 3-(2'-ethoxy-4'-diethylamino-phenyl) - 3 - (2' - methylindol - 3' - yl)-phthalide represented by the following formula



as a light-yellow color former having a melting point of 223–225° C. When a benzene solution of the color former was brought into contact with an acid clay layer coated on a paper, the color former immediately colored violet.

#### PRODUCTION EXAMPLE 8

20 A mixture of 2.0 g. of 1,2 - dimethyl - 3 - (2' - carboxy-benzoyl)-indole, 1.2 g. of N-acetyl-N-methyl-m-anisidine, and 20.0 g. of acetic anhydride was heated to 80–90° C. for 2 hours, with stirring, to cause the reaction. The reaction mixture was then treated as in Production Example 1 to provide 2.0 g. of 3-(2'-methoxy-4'-N-acetyl-N-methylamino-phenyl) - 3 - (1',2' - dimethylindol - 3' - yl)-phthalide represented by the following formula



as a white color former having a melting point of 245–253° C. When a benzene solution of the color former was brought into contact with an acid clay layer coated on a paper, the color former immediately colored violet-blue.

#### PRODUCTION EXAMPLE 9

45 A mixture of 2.2 g. of 1-ethyl-2-phenyl-3-(2'-carboxy-benzoyl)-indole, 1.4 g. of N-methyl-N-benzylamino-phenyl-m-anisidine, and 15.0 g. of acetic anhydride was heated to 80–90° C. for 2 hours, with stirring, to cause the reaction. Then, the reaction mixture was treated as in production Example 1 to provide 2.1 g. of 3-(2'-methoxy-4' - N-methyl-N-benzylamino-phenyl) - 3 - (1' - ethyl-2' - phenylindol - 3' - yl)-phthalide represented by the following formula



as a light-yellow color former having a melting point of 190–197° C. When a benzene solution of the color former was brought into contact with an acid clay layer coated on a paper, the color former immediately colored violet-blue.

The microcapsules used in the pressure-sensitive copying papers may be formed by any state of the art process used to form oil-containing pressure-sensitive microcapsules, e.g., as described in U.S. Pats. 2,548,366, 2,800,457 or 2,800,458. These processes utilize the phenomenon of composite coacervations.

The amount of the color former to be used is generally 0.5–5.0% by weight based on the weight of the organic solvent described above, such as ethylene glycol, chloro-

benzene, and chlorodiphenyl. However, lesser and greater amounts may be used.

As the electron accepting solid acid, acid clay, attapulgite, zeolite, bentonite, kaolin, acid polymers such as phenolic resin etc. are used.

The pressure-sensitive copying paper of this invention in which the phthalide compound represented by the aforesaid general formula is used as a color former is colorless or has a very faint yellow character before use, but when the pressure-sensitive copying paper subjected to localized pressure by, e.g., handwriting or typewriting, purple or blue coloring instantly occurs. Moreover, the color density of the color thus formed is high, and the light and water resistance thereof are excellent.

Furthermore, by using the aforesaid color former together with known yellow-color formers, red-color formers, blue-color formers, green-color formers, and the like, a pressure-sensitive copying paper capable of providing various colors copying can be obtained unaccompanied by any adverse effect, such as; desensitization.

The present invention will now be further explained in greater detail by the following examples.

#### Example 1

In 100 g. of trichlorodiphenyl there was dissolved 2.5 g. of 3-(2'-methyl - 4' - diethylaminophenyl)-3-(1',2'-dimethylindol-3'-yl)-phthalide, and then 20 g. of gum arabic and 160 g. of water were added to the solution at 50° C. followed by emulsification. To the emulsion were added 20 g. of acid-treated gelatin and 160 g. of water and thereafter the pH of the emulsion was adjusted to 5 by adding acetic acid while stirring. Then, 500 g. of water was added to the system to cause coacervation and to form dense liquid films of gelatin-gum arabic around the oil drops of trichlorodiphenyl. After adjusting the pH of the system to 4.4, 3.8 g. of aqueous 37% formalin solution was added thereto to harden the aforesaid liquid films. The system was then cooled to 10° C., the pH thereof was adjusted to 9 by adding an aqueous solution of sodium hydroxide, and the system was allowed to stand for 5-6 hours, whereby encapsulation was completed. The microcapsule-containing liquid was applied to a paper by roll coating or air-knife coating and dried to give a colorless coated sheet. When the coated paper (upper sheet) was placed on a sheet (lower sheet) having coated thereon a layer of acid clay (an electron accepting adsorbent) so that the microcapsule layer was closely brought into contact with the adsorbent layer and localized pressure was applied by handwriting or typewriting, the areas of the lower sheet to which pressure was applied were immediately colored blue.

The color density of the color former thus formed was high. Moreover when the blue color former was placed for an extended period of time in a chamber free from the direct rays of the sun, no discoloring was observed. When it was exposed to the direct rays of the sun for an extended period of time, fading was scarcely observed. Furthermore, the color former thus colored exhibited excellent water resistance.

On the other hand, when the same procedure as above was followed using a known color former, 3-(4'-dimethylaminophenyl)-3-(1',2'-dimethylindol-3'-yl)-phthalide, disclosed in U.S. Pat. No. 3,540,911, although the color former colored immediately blue-purple on the lower sheet, the color density was not high, and the light and water resistance thereof was poor.

#### Example 2

A colorless upper sheet was prepared following the same procedure as in Example 1 except that 1.5 g. of 3-(2'-ethoxy - 4' - diethylaminophenyl)-3-(1',2'-dimethylindol-3'-yl) phthalide was used as the color former. When the upper sheet was placed on the lower sheet so that the microcapsule layer was brought into intimate contact with the acid clay layer of the lower sheet and localized

pressure was applied thereto by handwriting, the areas of the acid clay layer thus pressed immediately colored violet-blue. Upon testing the violet-blue color former for light fastness, it was confirmed that the color former had sufficient stability for practical use. The violet-blue color former also was excellent in water resistance.

#### Example 3

A colorless upper sheet was prepared following the same procedure as in Example 1 except that 1.5 g. of 3-(2'-methoxy-4'-methylaminophenyl)-3-(1',2'-dimethylindol-3'-yl)-phthalide was used as the color former. When the upper sheet was placed on the lower sheet so that the microcapsule layer was brought into intimate contact with the acid clay layer of the under sheet and localized pressure was applied thereto by handwriting, the areas of the acid clay layer thus pressed immediately colored violet. By testing the color former thus colored violet with respect to light fastness, it was confirmed that the violet color former had sufficient stability for practical use.

#### Example 4

A colorless upper sheet was prepared following the same procedure as in Example 1 except that 1.5 g. of 3-(2'-methoxy - 4' - dimethylaminophenyl)-3-(1',2'-dimethylindol-3'-yl)-4,5,6,7-tetrachlorophthalide was used as the color former. When the upper sheet was placed on the lower sheet so that the microcapsule layer was brought into intimate contact with the acid clay layer of the lower sheet and localized pressure was applied thereto by handwriting, the areas of the acid clay layer thus pressed were immediately colored blue. By testing the blue color former with respect to light fastness, it was confirmed that the blue color former had sufficient stability for practical use.

35 The blue color former was also excellent in water resistance.

#### Example 5

A colorless upper sheet was prepared following the same procedure as in Example 1 except that 1.5 g. of 3-(2'-ethoxy - 4' - diethylaminophenyl)-3-(1',2'-dimethylindol-3'-yl)-5-dimethylaminophthalide was used as the color former. When the upper sheet was placed on the lower sheet so that the microcapsule layer of the upper sheet was brought into intimate contact with the acid clay layer of the lower sheet and localized pressure was applied thereto by handwriting, the areas of the acid clay layer thus pressed immediately colored violet-blue. By testing the violet-blue color former with respect to light fastness, it was confirmed that the violet-blue color former violet-blue had sufficient stability for practical use. The violet-blue color former was also excellent in water resistance.

#### Example 6

A colorless upper sheet was prepared following the same procedure as in Example 1 except that 2.0 g. of 3-(2'-ethoxy - 4' - diethylaminophenyl) - 3 - (1'-methyl-2'-phenylindol-3'-yl)-4,5,6,7-tetrabromophthalide was used as the color former. When the upper sheet was placed on the lower sheet so that the microcapsule layer of the upper sheet was brought into intimate contact with the acid clay layer of the lower sheet and localized pressure was applied thereto by handwriting, the areas of the acid clay layer that pressed immediately colored blue. By testing the blue color former with respect to light fastness, it was confirmed that the colored color former had sufficient stability for practical use. The colored color former also was excellent in water resistance.

#### Example 7

A colorless upper sheet was prepared following the same procedure as in Example 1 except that 2.0 g. of 3-(2'-ethoxy-4'-diethylaminophenyl)-3-(2' - methylindol-3'-yl)-phthalide was used as the color former. When the upper sheet was placed on the lower sheet so that the microcapsule layer of the upper sheet was brought into

intimate contact with the acid clay layer of the lower sheet and localized pressure was applied thereto by handwriting, the areas of the acid clay layer thus pressed immediately colored violet. By testing the violet color former with respect to light fastness, it was confirmed that the colored color former had sufficient stability for practical use.

Example 8

A colorless upper sheet was prepared following the same procedure as in Example 1 except that 2.0 g. of 3 - (2' - methoxy - 4' - N-acetyl-N-methylaminophenyl)-3-(1',2'-dimethylindol-3'-yl)-phthalide was used as the color former. When the upper sheet was placed on the lower sheet so that the microcapsule layer of the upper sheet was brought into intimate contact with the acid clay layer of the lower sheet and localized pressure was applied thereto by handwriting, the areas of the acid clay layer thus pressed immediately colored violet-blue. By testing the violet-blue color former with respect to light fastness, it was confirmed that the colored color former had sufficient stability for practical use.

Example 9

An upper sheet was prepared following the same procedure as in Example 1 except that 0.5 g. of 3-(2'-methoxy-4' - N - methyl - N - benzylaminophenyl)-3-(1'-ethyl-2'-phenylindol-3'-yl)-phthalide, 0.8 g. of o-hydroxybenzalacetophenone, 0.8 g. of Rhodamine B-Anilino-Lactam, 0.2 g. of Crystal Violet Lactone, and 0.2 g. of Malachite Green Lactone were used as the color formers. When the upper sheet was placed on the lower sheet so that the microcapsule layer was brought into intimate contact with the acid clay layer of the lower sheet and localized pressure was applied thereto by handwriting, the areas of the acid clay layer thus pressed immediately colored black. The color thus formed was very stable and had excellent light and water resistance.

What is claimed is:

1. A pressure-sensitive copying sheet comprising an adsorbent solid acid and a microencapsulated color former capable of forming a distinct color when reacted with said adsorbent solid acid coated on the same or different surface of support or supports, said microcapsules containing an organic solvent having dissolved therein a phthalide color former comprising at least one phthalide compound represented by the general formula



wherein R<sub>1</sub> represents a member selected from the group consisting of a hydrogen atom, a methyl group, an ethyl group, an acetyl group and a benzyl group; R<sub>2</sub> represents a member selected from the group consisting of a methyl group and an ethyl group; R<sub>3</sub> represents a member selected from the group consisting of a hydrogen atom,

a methyl group and an ethyl group; R<sub>4</sub> represents a member selected from the group consisting of a methyl group and a phenyl group; X represents a member selected from the group consisting of a methyl group, a methoxy group and an ethoxy group; Y represents a member selected from the group consisting of a hydrogen atom, a chlorine atom, a bromine atom and a dimethylamino group; and n is an integer from 1 to 4.

2. The pressure-sensitive transfer sheet as claimed in Claim 1 wherein said phthalide compound is selected from the group consisting of

- 3-(2'-methyl-4'-diethylaminophenyl)-3-(1',2'-dimethylindol-3'-yl)-phthalide,
- 3-(2'-ethoxy-4'-diethylaminophenyl)-3-(1',2'-dimethylindol-3'-yl)-phthalide,
- 3-(2'-methoxy-4'-methylaminophenyl)-3-(1',2'-dimethylindol-3'-yl)-phthalide,
- 3-(2'-methoxy-4'-dimethylaminophenyl)-3-(1',2'-dimethylindol-3'-yl)-4,5,6,7-tetrachlorophthalide,
- 3-(2'-ethoxy-4'-diethylaminophenyl)-3-(1',2'-dimethylindol-3'-yl)-5-dimethylaminophthalide,
- 3-(2'-ethoxy-4'-diethylaminophenyl)-3-(1'-methyl-2'-phenylindol-3'-yl)-4,5,6,7-tetrabromophthalide,
- 3-(2'-ethoxy-4'-diethylaminophenyl)-3-(2'-methylindol-3'-yl)-phthalide,
- 3-(2'-methoxy-4'-N-acetyl-N-methylaminophenyl)-3-(1',2'-dimethylindol-3'-yl)-phthalide, and
- 3-(2'-methoxy-4'-N-methyl-N-benzylaminophenyl)-3-(1'-ethyl-2'-phenylindol-3'-yl)-phthalide.

3. The pressure sensitive transfer sheet as claimed in Claim 1 wherein from about 0.5 to about 5.0% of said color former is present in said organic solvent based on the weight of said organic solvent.

4. The pressure-sensitive transferring sheet as claimed in Claim 1, wherein said microcapsules contain a least one color former in addition to said phthalide color former.

5. The pressure sensitive transfer sheet as claimed in Claim 4, wherein said at least one color former is selected from the group consisting of o-hydroxybenzalacetophenone, Rhodamine B-anilinolactam, Crystal Violet Lactone and Malachite Green Lactone.

References Cited

UNITED STATES PATENTS

|           |         |                     |          |           |
|-----------|---------|---------------------|----------|-----------|
| 3,540,911 | 11/1970 | Chao-han Lin        | -----    | 117-36.2  |
| 3,540,910 | 11/1970 | Chao-han Lin        | -----    | 117-36.8  |
| 3,713,863 | 1/1973  | Chao-han Lin et al. | 117-36.8 |           |
| 3,491,112 | 1/1970  | Chao-han Lin        | -----    | 117-36.2  |
| 2,505,486 | 4/1950  | Green               | -----    | 260-343.3 |
| 3,244,549 | 4/1966  | Farnham et al.      | -----    | 117-36.2  |
| 3,268,537 | 8/1966  | Gosnell et al.      | -----    | 117-36.2  |
| 3,336,337 | 8/1967  | Gosnell             | -----    | 117-36.2  |
| 3,455,721 | 7/1969  | Phillips et al.     | -----    | 117-36.2  |
| 3,491,111 | 1/1970  | Lin                 | -----    | 117-36.2  |

WILLIAM D. MARTIN, Primary Examiner

W. R. TRENOR, Assistant Examiner

U.S. CL. X.R.

117-36.2, 115 L, UA; 260-235, 240 G, 343.3